

## UNITED STATES PATENT OFFICE.

PAUL D. MERICA, OF NEW YORK, N. Y., AND THOMAS H. WICKENDEN, OF BOSEILLE, NEW JERSEY, ASSIGNORS TO THE INTERNATIONAL NICKEL COMPANY, OF NEW YORK, N. Y., A CORPORATION OF NEW JERSEY.

## ADDITION MATERIAL FOR FERROUS METALS.

No Drawing.

Application filed March 10, 1924. Serial No. 698,284.

Our invention relates to the adding of nickel to cast irons or steels, and is designed especially to overcome the difficulty arising from the high melting point of nickel, particularly as compared to cast iron and other ferrous metals.

In adding nickel to cast iron the addition has usually been made in the ladle rather than in the melting cupola, inasmuch as the nickel cast iron is usually only a part of the cupola production. When ordinary nickel is added to the molten cast iron in the ladle, it has been difficult to prevent segregation on account of incomplete melting of the nickel, and also in some cases there has been a tendency to produce blow-holes. Our invention is designed to overcome these difficulties which are due mainly to the fact that cast iron melts at a much lower temperature than nickel and to the introduction of a small amount of oxygen or oxide with the nickel. The invention consists in uniting with the nickel previous to its addition to the ferrous metal a substance or substances which will lower the melting point of the nickel, and which will have no deleterious action upon the ferrous metal to which the nickel is added.

Commercial cast iron contains usually from .75 to 3.5 per cent of silicon, from .10 to 1.5 per cent of phosphorus and from 2.5 to 4 per cent of carbon, with certain other metalloids.

Inasmuch as carbon and silicon are present in the cast iron and also serve to lower the melting point of nickel, we prefer to employ these two materials for adding to the nickel, and we prefer to add to the nickel from .25 to 2.5 per cent of carbon, and from 1 to 10 per cent of silicon. In practice, we have successfully employed from 2 to 6 per cent of silicon and about  $\frac{3}{4}$  to 1 per cent of carbon in the nickel, and the nickel thus combined has a melting point sufficiently near cast iron so that it is well melted and dissolved in the cast iron and an excellent cast iron nickel alloy produced. We have often used about 5 per cent of nickel thus treated as the addition to the cast iron. It will be noted that with the preferred amounts of silicon and carbon added to the nickel, there is no material change in the percentages of these metalloids in the final cast iron nickel

alloy, and we preferably make the additions to the nickel in such percentages that there is no material change in the metalloid percentages of the cast iron. This is one of the advantages of adding materials to the nickel which do not materially change the analysis of the cast iron itself. The effect of the silicon and carbon is also of advantage in that their presence tends to eliminate any traces of oxides in the nickel addition, which oxides might react with the carbon of the iron to produce blow-holes.

We have also added aluminum to the nickel along with the carbon and silicon. The aluminum also serves to further slightly decrease the melting point and prevent any trace of oxidation. It also has a deoxidizing effect on the ferrous metals of which the nickel is made. When this material is added to the iron it also tends to produce a noticeable amount of heat by chemical reaction which tends to sustain the temperature of the molten iron and provide a longer time for the solution of the nickel. The aluminum is preferably added to the nickel in a percentage of .1 to 5 per cent, and we have added 1 per cent with good results.

The nickel alloy is preferably formed into shot before adding to the cast iron or ferrous material, if it is to be added to a molten bath. When aluminum is added to the nickel alloy, it tends to change the form of the shot from round globules to small feathery particles having a greater ratio of surface to volume and hence giving more rapid dissolving in the iron.

The additions to the nickel may be made in any desirable manner, for example, the silicon may be added in the form of ferro-silicon, and the carbon in the form of either flour carbon or tar coke.

The nickel with the artificially lowered melting point caused by the additions to it may be added to the cupola in the form of a small ingot mixed with the cupola charge, and thereby melt along with the cast iron in the cupola, where the entire cupola charge is to be used in alloy form.

Phosphorus may be added to the nickel with or without the other additions named, but should be used only in limited amounts and in special cases where it will have no deleterious effect on the ferrous metal to

which the nickel material is added. Where we have used the high-carbon low-silicon shot we have gotten good results from a shot which will pass through a  $\frac{1}{4}$  inch screen. 5 Magnesium may also be used either with or without the other additions to the nickel to lower its melting point, and other variations may be made without departing from our invention, since we consider ourselves the 10 first to add to a ferrous material nickel having an artificially lowered melting point to give better solution and mixing in the alloy.

We claim:

1. As an addition material for molten cast 15 iron baths, metallic nickel having alloyed therewith another material sufficient in percentage to lower the melting point of the alloy to substantially that of cast iron.

2. As an addition material for molten cast 20 iron, metallic nickel having alloyed therewith metalloid material sufficient in amount to lower the melting point of the alloy to substantially that of cast iron.

3. In the manufacture of cast iron containing 25 nickel, the step consisting of adding to a bath of molten cast iron metallic nickel having alloyed therewith another material sufficient in amount to lower the melting point of the alloy to substantially that of cast iron.

4. In the manufacture of cast iron containing nickel, the step consisting of adding to the bath of molten cast iron, metallic 35 nickel in solid form and having alloyed therewith metalloid material sufficient in amount to lower the melting point of the alloy to substantially that of the cast iron.

5. In the manufacture of cast iron containing nickel, the step consisting of adding 40 to a bath of molten cast iron metallic nickel in divided form and having alloyed therewith metalloid material sufficient in

amount to lower the melting point of the latter to substantially that of cast iron.

6. In the manufacture of cast iron containing 45 relatively small proportions of nickel, the step consisting of adding to a bath of molten cast iron a nickel alloy containing metallic nickel as its major ingredient and also containing metalloid material 50 sufficient in amount to lower the melting point of the alloy to substantially that of the cast iron.

7. In the making of a ferrous alloy, the 55 step consisting of adding to ferrous material containing iron as a predominant element nickel containing carbon .25% to 2.5% and silicon from 1% to 10%.

8. As an addition material for ferrous 60 materials containing iron as a predominant element nickel containing carbon .25% to 2.5% and silicon from 1% to 10%.

9. In the making of a ferrous alloy, the 65 step consisting of adding to ferrous material containing iron as a predominant element, nickel containing carbon .25% to 2.5%, silicon from 1% to 10% and aluminum from 1% to 5%.

10. As an addition material for ferrous 70 materials containing iron as a predominant element, nickel containing carbon .25% to 2.5%, silicon from 1% to 10% and aluminum from 1% to 5%.

11. As an addition material for ferrous 75 material containing iron as the predominant element, nickel having added thereto a metalloid non-injurious to iron and sufficient in amount to lower the melting point of the nickel to substantially that of cast iron.

In testimony whereof we have hereunto 80 set our hand.

PAUL D. MERICA.  
THOMAS H. WICKENDEN.